

April 13, 1926.

1,580,198

H. C. HARRISON

## PROCESS OF PRODUCING COATED OR OTHER THIN METALLIC SHEETS

Filed May 21, 1925

2 Sheets-Sheet 1



Fig. 1.



Fig. 5.



Fig. 2.

Inventor

Herbert C. Harrington,

By Spencer, Sewall & Hardman  
Attorneys.

1,580,198

April 13, 1926.

H. C. HARRISON

PROCESS OF PRODUCING COATED OR OTHER THIN METALLIC SHEETS

Filed May 21, 1925

2 Sheets-Sheet 2



Fig. 3.



Fig. 4.



Inventor

Fig. 6. Herbert C. Harrison,

By Spencer, Lewall & Hardman,  
Attorneys.

Patented Apr. 13, 1926.

## UNITED STATES PATENT OFFICE.

HERBERT CHAMPION HARRISON, OF LOCKPORT, NEW YORK.

## PROCESS OF PRODUCING COATED OR OTHER THIN METALLIC SHEETS.

Application filed May 21, 1925. Serial No. 31,921.

*To all whom it may concern:*

Be it known that I, HERBERT CHAMPION HARRISON, a subject of the King of Great Britain and Ireland, residing at the city of Lockport, in the county of Niagara and State of New York, have invented certain new and useful Improvements in Processes of Producing Coated or Other Thin Metallic Sheets, of which the following is a full, 10 clear, and exact description.

This invention relates to the manufacture of thin sheets of ductile metal, such as copper, and, more specifically, to a process, including an electrolytic step, for making 15 metallic sheets having a protective film or coating on one side only.

In the production of metallic sheets electrolytically, it has been customary to perform such finishing operations upon the 20 sheets as are deemed necessary after the sheets have been stripped from the cathode surfaces.

I have found that electrolytically produced sheets may be more economically and 25 conveniently finished, for many purposes, before they have been stripped from the cathode, and that a burnishing treatment applied to the deposited layers on the 30 cathode will accomplish the further useful function of loosening the layer from the cathode, and will facilitate the stripping operation.

Furthermore, there are many uses for thin 35 sheets, as of copper, coated on one side only with a thin film of protective material, such as tin, zinc or lacquer. For example, in making radiators for motor vehicle engines, it is highly desirable to use thin copper strips of about five one-thousandths of an 40 inch in thickness, and approximately three to four inches in width, which are coated with tin. The tin coating facilitates the dipping process by which the contacting surfaces of the radiator elements are soldered or metallically united, and made 45 water-tight. Surfaces of radiator elements coated with tin offer great resistance to corrosion by alkaline water which so frequently is used in the cooling system of the 50 motor vehicle engine. There is, however, no advantage in tinning the strips on both sides. Only the side in contact with the circulating water of the cooling systems needs this protection. Hence all the advantages obtainable from tinning the radiator 55

elements is realized by tinning one side of the strip. If, therefore, a cheap, commercially workable method of tinning sheets on one side only is available, a considerable benefit would accrue in the more economical 60 production of tin-coated radiators.

The practical difficulties of applying a coat of tin to one side only of a sheet at a cost low enough to render it available for ordinary demands have never, to my knowledge, been overcome.

By the method hereinafter described, thin sheets of copper, having a film of tin on one side, may be produced by depositing copper electrolytically upon a sheet metal cathode, 70 dipping the compound sheet thus formed in a tinning bath, then burnishing the tinned surfaces by giving said compound sheet a progressive working operation sufficient to burnish the surfaces of the layers and loosen 75 the layers from the cathode, and then stripping the layers from the cathode sheet to form two sheets of thin copper, each having a thin film of tin on one side only.

In the accompanying drawings, in which like reference characters indicate like parts throughout the several views:

Fig. 1 is a diagrammatic illustration of an electrolytic apparatus for depositing metallic layers upon both sides of a cathode sheet 85 of indefinite length;

Fig. 2 is a diagrammatic illustration of an apparatus for coating the compound sheet produced in the electrolytic apparatus;

Fig. 3 is a diagrammatic illustration of 90 one apparatus for burnishing and stripping the electrolytically deposited layers to form two thin sheets;

Fig. 4 is a diagrammatic illustration of a preferred apparatus for accomplishing the 95 same result as the apparatus shown in Fig. 3;

Fig. 5 is a view of the electrolytic cell shown in Fig. 1, viewed from the left; and 100

Fig. 6 is a side view of rolls shown in 105 Fig. 4.

In Fig. 1, numeral 10 indicates an electrolytic cell beneath which is a catch-pan 11, adapted to receive electrolyte flowing from the cell. In this diagram the electrolyte is indicated as being continuously circulated from the tank 12, through pipe 13 into one end of the cell 10, and out from said cell through openings that admit the passage of 110 the thin traveling cathode sheet or ribbon

15, into the pan 11, whence it is pumped by an acid-proof pump 14 through pipe 16 to tank 12, thus completing the circuit. In this diagram, 17 indicates a spool from 5 which the ribbon cathode is unwound, and 18 a mechanically-driven reel by which the ribbon cathode may be drawn from the spool 17 (which may, if desired, be so mounted as to apply tension to the ribbon), 10 through the cell at any regulated speed necessary. Suitable connections between the anode and cathode and a source of current, (not shown) may be made at 19 and 19<sup>a</sup> respectively; the latter necessarily being in 15 the form of a brush or "slip" connection. The compound sheet consisting of the cathode ribbon and deposited layers, is indicated at 15<sup>a</sup>.

After the entire length of the cathode ribbon has been plated with a layer, say five 20 one-thousandths of an inch thick, or of any suitable thickness, the roll of compound sheet or strip 15<sup>a</sup>, consisting of the cathode strip sandwiched between two deposited layers, 25 may be placed upon another reel or spool, and said compound strip unwound therefrom and passed progressively through a bath of liquid coating material, and then the layers may be burnished progressively 30 and stripped; or, in the event that it is not desired to produce sheets coated with a protecting film on one side, the roll of compound strip may be placed upon a spool, the end passed between working and burnishing 35 instrumentalities, and the strip then subjected progressively to a burnishing, layer-loosening and stripping process. The edges of the compound strip may, if desired, be sheared or otherwise trimmed, but it is preferred to crack or weaken the bond between 40 the layers at the edges by working the strip.

If it is desired to produce, for example, tin-coated sheets of metal, the roll of compound strip or sheet 15<sup>a</sup> may be placed upon 45 a delivery spool 20, as indicated in Fig. 2, and lead into and through a suitable fluxing bath 21, around guide-rolls 22, and thence into and through a tinning bath 23, around guide-rolls 24. From the tinning bath, the 50 compound sheet, now having a coating of tin and designated by 15<sup>b</sup>, is led between suitable scrapers or "doctors" 25, and squeezing rolls 26, to remove excess of coating from the compound strip 15<sup>b</sup> and direct such excess back into the bath, as is usual. The strip 15<sup>b</sup> may then be led over a guide-roll 55 27 and finally wound upon a spool 28.

For the purpose of burnishing the surfaces of the strip or sheet 15<sup>b</sup> or 15<sup>a</sup>, whether 60 it be coated with a protecting film or not, and loosening the adhesion of the layers, a roll of said compound strip may be placed upon a delivery reel or spool 30, and one end led through the pass of a pair of plain faced rolls 31, set to exert a pinch upon the

compound strip sufficient to burnish its surface and apply enough reducing or working pressure to cause a slight localized molecular flow adequate to loosen the adhesion of the layers to the cathode strip, and sufficient to 70 crack and weaken or sever the bond between the layers upon opposite sides of the cathode strip where they unite around its edges. The loosened layers may be peeled from the cathode strip after the advance end has been 75 fed through the roll pass and between the guides 32, and each stripped layer 15<sup>c</sup>, as an independent sheet, may be attached to a winding reel 33. The advance end of the cathode strip 15 from which the deposited 80 layers have now been separated, may be attached to reel 34. Now, as the compound strip transverses the roll pass, drawn through it by the bite of the revolving rolls 85 upon it, the stripping reels 33 may be caused to strip the layers 15<sup>c</sup> from the cathode sheet 15, and wind them into coils; and the reel 34 may assist the passage of the compound strip through the roll pass, and wind the cathode strip in a roll of cathode strip suitable to be 90 used again to receive a new deposit in the electrolytic cell.

A preferred method of loosening the layers is to work the layers by repeatedly flexing the compound strip. There are many 95 instrumentalities whereby this may be accomplished. In Fig. 4 one means is shown for thus working the compound strip to loosen the layers and at the same time burnish their outer surface. In Fig. 4, 30<sup>a</sup> indicates a roll or spool of compound strip, 15<sup>a</sup> or 15<sup>b</sup>, consisting of a cathode core plated with layers of copper, for example, either coated or uncoated. The compound strip may be threaded between bars or rolls 31<sup>a</sup> 100 staggered with respect to each other and adjusted to cause the strip to assume a wavy or zigzag form between them. The bars or rolls 31<sup>a</sup> may be arranged in two series, which may be adjusted toward or from 105 each other. The compound strip may be drawn from the spool between the bars or rolls 31<sup>a</sup> thereby progressively flexing it 110 repeatedly in opposite directions during its progress, thus loosening the layers from the 115 cathode strip and weakening or cracking the bond between the layers at the edge of the compound strip by working the layers so that the layers may be readily stripped from the cathode. The stripped layers may 120 be separately wound, as sheets of copper 15<sup>c</sup> (coated or uncoated), on revolving spools or reels 33<sup>a</sup>, while the cathode core of the compound sheet is being wound on reel 34<sup>a</sup> and drawn between the rolls or bars of the working 125 instrumentality.

If desired, in order to draw or assist in drawing the compound strip through or between the flexing elements 31<sup>a</sup>, the sheet 130 may be subjected to pressure between pinch

rolls 35, which may have the additional function of further weakening or cracking the bond between the layers 15° at the edges of the compound strip. The rolls 35 may be so formed as to apply pressure only to the edges of the compound sheet if desired, as indicated in Fig. 6.

The rubbing or rolling pressure on the outer surfaces of the compound strip as it 10 is being drawn between the working elements will have a burnishing effect if the adjustment of said elements is such that adequate friction is applied.

A cathode strip of copper eight inches in 15 width, five one-thousandths of an inch in thickness and of indefinite length, has been found suitable for the purpose. In the manufacture of copper sheet for use in radiators these dimensions are desirable because they are those of standard rolled stock 20 used in manufacture and when damaged by use as cathodes they can be cut up and used for making radiating elements. Although it is possible to strip the deposit from a highly 25 burnished metallic cathode surface, it may be desirable to apply a coating to the surface before subjecting it to the electrolyte. Many kinds of coating material are known for this purpose. I have found sodium 30 sulphide a satisfactory cathode coating material.

Although the process of this invention has been described and illustrated for the purpose of disclosing in detail one useful application of the invention, it is not intended to be limited to a particular kind of deposited metal or a particular kind of coating film, as the principle of the invention has a much broader application.

40 What I claim and desire to secure by Letters Patent of the United States is as follows:

1. The method of producing thin metallic sheets which comprises depositing a layer 45 of ductile metal electrolytically upon a cathode sheet, then subjecting the compound sheet thus formed to a working operation applied progressively, thereby loosening the deposited layer from the cathode sheet, and 50 then stripping the layer from the cathode sheet.

2. The method of producing thin metallic sheets, which comprises depositing a layer 55 of ductile metal electrolytically upon a cathode sheet, then subjecting the compound sheet thus formed to working by progressively flexing it in opposite directions, thereby loosening the layer from the cathode sheet.

60 3. The method of producing thin metallic sheets which comprises depositing a layer 65 of ductile metal electrolytically upon each side of a cathode sheet, then subjecting the compound sheet thus formed to a working operation applied progressively, thereby

loosening the deposited layers from the cathode sheet, and then stripping both layers from said cathode sheet.

4. The method of producing thin metallic sheets which comprises depositing an envelope 70 of ductile metal electrolytically around a cathode sheet, then subjecting the compound sheet thus formed to a working operation applied progressively, thereby loosening the layers of the envelope adhering 75 to the surfaces of the cathode sheet and cracking the connecting bond at the edges

5. The method of producing thin metallic sheets which comprises progressively depositing an envelope of ductile metal around 80 an elongated flexible cathode by causing it to progress from end to end through an electrolytic bath, progressively severing the envelope on the cathode longitudinally into two layers, then stripping said layers from 85 the flexible cathode.

6. The method of producing thin metallic sheets which comprises depositing an envelope 90 of ductile metal electrolytically around a cathode sheet, then subjecting the compound sheet thus formed to working by progressively flexing it in opposite directions, thereby loosening the layers of the envelope adhering to the surfaces of the cathode sheet and cracking the connecting 95 bond at the edges.

7. A method of producing thin metallic sheets having a protective coating on one side, which comprises depositing a layer of 100 metal electrolytically upon a cathode, dipping the body so formed into a bath of liquid coating material, and stripping the metallic, coated layer from the cathode.

8. A method of producing thin metallic sheets having a protective coating on one side, which comprises depositing a layer of 105 metal electrolytically upon a cathode sheet, dipping the compound sheet so formed into a bath of liquid coating material, and stripping the metallic, coated layer from the 110 cathode sheet.

9. A method of producing thin metallic sheets having a protective coating on one side, which comprises depositing a layer of 115 metal electrolytically upon each side of a cathode sheet, dipping the compound sheet so formed into a bath of liquid coating material, and stripping the metallic, coated layers from the cathode sheet.

10. A method of producing thin metallic sheets having a protective coating on one side, which comprises depositing an envelope 120 of metal electrolytically around a cathode sheet, dipping the compound sheet thus formed in a bath of liquid coating material and then cracking the envelope at its edges and stripping the surface layers from said cathode sheet.

11. A method of producing thin metallic sheets having a protective coating on one 130

side, which comprises depositing an envelope of metal electrolytically around a cathode sheet, dipping the compound sheet thus formed in a bath of liquid coating material, severing the envelope while on the cathode sheet into two layers, one on each side of the cathode sheet, and stripping the severed layers from said cathode sheet.

12. A method of producing thin metallic sheets having a protective coating on one side, which comprises depositing a layer of ductile metal electrolytically upon a cathode sheet, dipping the compound sheet thus formed into a liquid bath of suitable protective material, then subjecting the compound, coated sheet to a working operation progressively applied, thereby burnishing the metallic coating and loosening the layer from the cathode sheet, and then stripping the coated layer.

13. A method of producing thin metallic sheets having a protective coating on one side, which comprises depositing a layer of ductile metal electrolytically upon a cathode sheet, then treating the surface of the layer to cause adhesion of a metallic coating, dipping the compound sheet thus formed into a liquid bath of suitable protective metal, then subjecting the compound coated sheet

to a working operation progressively applied, thereby burnishing the metallic coating and loosening the layer from the cathode sheet, and then stripping the coated layer therefrom.

14. A method of producing thin metallic sheets having a protective coating on one side, which comprises depositing an envelope of ductile electrolytically around a cathode sheet, dipping the compound sheet thus formed in a liquid bath of suitable coating metal, then subjecting the compound sheet to a working operation progressively applied, thereby burnishing the metallic coating, loosening the layers of the envelope from the surfaces of the cathode sheet and cracking the connecting bond of the envelope at the edges, and finally stripping the layer from the cathode sheet.

15. A method of producing thin metallic sheets by progressively depositing metal electrolytically upon a cathode in a coherent layer, then stripping the layer from said cathode in the manner substantially as described.

In testimony whereof, I hereto affix my signature.

HERBERT C. HARRISON.